

1

2,957,478

## METHOD OF MAKING A SMOKING PRODUCT

Eric Bell Hotelling and Thomas Edward Kelly, Westport, Conn., assignors to International Cigar Machinery Company, Inc., a corporation of New Jersey

No Drawing. Filed Sept. 30, 1959, Ser. No. 843,376

6 Claims. (Cl. 131—140)

This invention relates to tobacco compositions containing finely divided tobacco, a water-insoluble adhesive derived from a polysaccharide and a polyester plasticizer. The invention further relates to articles such as sheets and filaments manufactured from such compositions and to methods of making both the compositions and the articles.

In forming and wrapping cigars and related smoking articles it is important that the tobacco material on the outside should stretch and cling resiliently to the filler or bunch on the interior as a close fitting skin. Some natural leaf tobacco has this property. It is of substantial technical value to be able to use manufactured tobacco sheets for the same purposes. Sheet and filament products of finely divided tobacco not only have economic and mechanical advantages in their ease of automatic manipulation and saving on scrap, but also provide a means of blending different tobaccos.

An important consideration in formulation of tobacco sheet compositions is a close approach to the quality of natural leaf tobacco in flavor and smoke as well as burn rate and ash formation. These factors are influenced by the selection of suitable adhesives and plasticizers which are generally used in minimal amounts commensurate with strength and stretch. The tobacco content is therefore made as high as possible.

There is an inherent advantage in tobacco sheet and related products which have high resistance to attack by moisture, such as saliva and casing fluids. Accordingly, various systems have been developed for forming such articles from combinations of finely divided tobacco and water-insoluble ingredients, such as adhesives, which are manipulated in organic solvents.

An outstanding problem, not resolved or suggested in the prior art, is the production of tobacco sheet having not only good color, strength (both wet and dry), and burn properties but also a high stretch or plasticity in combination with a high tobacco content (greater than two thirds by weight).

Therefore, it is an object of this invention to provide a tobacco composition from finely divided tobacco and a highly stretchable water-insoluble adhesive in combination with a plasticizer.

It is a further object to provide a tobacco sheet or filament having a high tobacco content, water insolubility and high stretch.

Another object of the invention is to provide smoking articles including cigars which are made at least in part from finely divided tobacco combined with a water-insoluble adhesive which contains a high stretch ingredient.

Still another object of this invention is to provide methods of manufacturing tobacco compositions and articles from finely divided tobacco in organic solvent systems.

These and other objects of the invention are more fully

2

set forth in the following detailed description and examples.

This invention is preferably realized by contacting finely divided tobacco with a water-insoluble adhesive dissolved in an organic liquid solvent in combination with the polyester plasticizer materials of the invention. It has been found that a rather specific group of polyesters adds valuable stretch properties to tobacco products when used in small amounts. Moreover, these materials do not seem to impair either the smoke or burning properties of the tobacco and further serve as auxiliary adhesives.

The ester polymers of this invention are prepared by combined dicarboxylic acids with aliphatic triols (straight chain alcohols containing three hydroxy groups). In selecting the desirable acids and alcohols to be used in this invention it is important to avoid heavy cross linking, through condensation, and the resulting rigid, infusible and insoluble alkyd materials. The desired polyester materials are probably slightly cross linked and are gummy. The polyesters of this invention may also be mixed and used with other plasticizers such as esters of dihydroxy alcohols including the glycols and with conventional humectants. These products are useful both as plasticizing and as adhesive materials.

The aliphatic long-chain dicarboxylic acids useful in this invention include glutaric acid, adipic acid, pimelic acid, suberic acid, azelaic acid, sebatic acid, their higher homologues, and acids of this type which are substituted with lower alkyl groups.

A preferred embodiment of this invention utilizes polyesters prepared from mixtures of azelaic acid or sebatic acid with a dicarboxylic acid of shorter chain length to produce a mixed dicarboxylic acid with an average chain length of 7-9 carbon atoms. Dicarboxylic acids with chain lengths of less than five carbon atoms tend to produce rigid structures which are not useful in this invention. Certain of the dicarboxylic acids, succinic, adipic and suberic acids, produce solvent-insoluble polyesters when condensed in purified form with glycerol or other triols. It is preferable, therefore, to employ these acids as crude technical mixtures with other dicarboxylic acids or, if the purified acids are available, to add azelaic or sebatic acids to the reaction mixture to produce a lower-melting, less highly cross-linked polyester which will dissolve. Substitution of these acids with lower alkyl group (methyl or ethyl) also greatly reduces their tendency to resinify. A particularly suitable dicarboxylic acid technical raw material is "Isosebatic Acid," a commercial mixture of about 10% sebatic acid, about 60% 2-ethylsuberic acid and about 30% 2, 5-diethyladipic acid by weight.

Any aliphatic triol containing vicinal hydroxyl groups, which inhibit the cross-linking reaction, is useful in forming the polyesters of this invention. Preferred species of triol include glycerol and 1, 2, 6-hexanetriol. Glycerol is particularly preferred because it is cheap, readily available and non-toxic.

The mole ratio of dicarboxylic acid to triol is critical and is at least 2:1 and not more than 3:1. Less than two moles of acid per mole of glycerol cause resinification, in most cases, to an insoluble alkyl-type polymer. Use of more than three moles of acid to one mole of glycerol leaves a residue of unreacted acid which tends to produce a fatty odor in the tobacco product.

Polyesters useful in this invention are produced by condensation of the dicarboxylic acids and glycols above within these proportions. The condensation can be carried out by any of the usual commercial or laboratory

methods of esterification. One of the simplest procedures is to dissolve or suspend the reactants in benzene or toluene, add a few percent of concentrated sulfuric acid or phosphoric acid as catalyst, distill off the water formed in the reaction as an azeotrope with the benzene or toluene, and collect the water in a trap for azeotropic removal of water with provision for the benzene or toluene to reflux into the reaction vessel. When evolution of water ceases, generally after three to twelve hours at reflux temperature, the condensation is essentially complete. The polyester may conveniently be employed in the crude benzene or toluene solution after separation of the acid catalyst, or it may be further purified if desired.

The benzene or toluene solution is fully stable for periods of several months if water is excluded and the acid efficiently separated from the organic layer. In an alternate method, the benzene may be distilled off in vacuo and the gummy polyester taken up in another suitable solvent such as methanol, ethanol or acetone. If rigid exclusion of acids is desired, the condensation may be carried out in a higher-boiling solvent, or under pressure, without any catalyst other than an excess of dicarboxylic acid reactant.

The polyesters of this invention function as both plasticizers and auxiliary adhesives with tobacco. Formulations containing them can tolerate a much higher tobacco loading than equivalent formulations plasticized with other materials.

The choice of the water-insoluble adhesive to be employed in preparing the tobacco products of this invention is subject to certain limitations. The material should be nearly tasteless and completely nontoxic in the concentrations used, should possess good burn odor, should be virtually insoluble in water but soluble in whatever organic solvent is chosen for the process to form a viscous solution which can be cast, sprayed or extruded, and from economic considerations should be inexpensive and readily available.

These limitations indicate the choice of the ester or ether derivatives of polysaccharide or carbohydrate high polymers such as cellulose, amylose and starches. Such materials, which are in widespread use, include cellulose esters, particularly cellulose acetate, the mixed esters such as cellulose acetate propionate and cellulose acetate butyrate, and cellulose ethers such as methylcellulose and ethylcellulose. The molecular weight and degree of substitution of the cellulose or other carbohydrate derivative must be in the proper range to produce the solubility and viscosity characteristics mentioned above. Within these limitations the particular adhesive chosen will depend upon the specific flavor, burn odor and texture which the formulator wishes to impart to the finished smoking article. The preferred adhesives in formulations containing the polyesters of this invention are ethers of cellulose or amylose.

The solvent chosen for the manufacture of tobacco products of this invention must be one that dissolves the adhesive, evaporates easily and is preferably cheap and easily recoverable. High-speed drying at slightly elevated temperatures is desirable. Among the common solvents it is preferable to employ methanol, but acetone, ethanol, isopropyl alcohol, benzene, toluene, chloroform and methyl butynol or mixtures of any of these can be used with particular adhesives and polyesters which dissolve in the solvent chosen.

#### Example I

This example illustrates a preferred form of the invention.

A plasticizer solution was prepared from 3058 grams (15.1 moles) of "Isobasic Acid" (a commercial mixture of sebamic acid, 2-ethylsuberic acid, and 2,5-diethyladipic acid), 507 grams (5.5 moles) of glycerol, 107 g. (3% by weight of reactants) of concentrated sulfuric acid

(specific gravity about 1.84), and 7.0 liters of benzene. These ingredients were stirred and refluxed in a 22-liter, four-neck, round-bottom flask equipped with a motor stirrer, thermometer well, heating mantle, two reflux condensers and two modified Dean-Stark traps for collection of water. After refluxing with stirring for a total of ten hours, the theoretical amount of water was collected from the traps and no further reaction was visible. The benzene solution of crude polyester was then separated from the lower acid layer. The polyester content, determined by drying a sample to constant weight, was 40%.

Ten grams of ethylcellulose (a commercial product described as having a medium ethoxy content and a viscosity of 100 cps. measured in solution under standard conditions) were dissolved in 200 ml. of methanol. Then 5.0 grams of the benzene solution of polyester, containing 2.0 grams of active material, were added to the solution and completely dispersed in it. This was followed by 60.0 grams of dry ball-milled Havana Seed Tobacco, all of which had passed through a 170-mesh screen. The thick slurry was adjusted to 27% solids content by addition of more methanol and, after complete homogenization, was cast into sheets with a casting knife clearance of about six mils. The solvent was permitted to evaporate at room temperature and atmospheric pressure, and random samples of the sheets were removed for testing. The sheet tensile strength was over 450 grams per inch for a sheet weight of 5.90 grams per square foot. After soaking in water for 30 seconds the tensile strength of this sheet was still over 250 grams per inch, and the elongation at the breaking point was over 15%.

Cigarillos prepared on a cigarillo machine with this tobacco sheet as wrapper were quite satisfactory in taste and appearance. The wrapper contained over 83% tobacco and less than 2.8% polyester by weight on a dry basis.

#### Example II

To illustrate the effects of changing the proportion of ingredients, a number of tobacco sheets were prepared from the polyester of Example I combined with ethylcellulose and tobacco in varying proportions by the procedure of Example I. The following data were obtained:

| Sheet | Ethylcellulose, g. | Polyester, g. | Tensile Strength, g./in. |     |     |                     |
|-------|--------------------|---------------|--------------------------|-----|-----|---------------------|
|       |                    |               | Tobacco g. (Percent)     | Dry | Wet | Elong., Wet Percent |
| A     | 10                 | None          | 60 (86%)                 | 565 | 245 | 10                  |
| B     | 10                 | 1             | 60 (85%)                 | 425 | 250 | 11                  |
| C     | 10                 | 2             | 60 (83%)                 | 440 | 275 | 16                  |
| D     | 10                 | 2             | 70 (85%)                 | 410 | 202 | 14                  |
| E     | 10                 | 2             | 50 (71%)                 | 590 | 400 | 19                  |
| F     | 10                 | 2             | 40 (77%)                 | 820 | 530 | 21                  |

Two conclusions may be drawn from this data. Sheets A, B, and C contain the same amounts of tobacco and ethylcellulose with variable amounts of polyester. Both the wet strength and the wet elongation of the sheets increases with increasing polyester concentration, indicating that the polyester functions both as a plasticizer and as an auxiliary adhesive. Secondly, sheets C, D, E, and F are composed of identical amounts of adhesive and polyester with variable quantities of tobacco. It is apparent that the tensile strength and elongation both decrease with increasing tobacco content, becoming marginal for cigarillos at about 85% tobacco.

#### Example III

A polyester solution was prepared by the procedure 75 of Example I from technical azelaic acid (2.75 moles)

and glycerol (1.0 mole) in toluene as the solvent and azeotroping medium. A portion of the product (2.0 grams, dry basis) was dissolved in methanol and mixed with 10.0 grams of ethylcellulose and 60 grams of tobacco to form a slurry with a solids content of 27%. Sheets cast from this slurry with an eight-mil knife had the following properties:

|                       |                     |      |
|-----------------------|---------------------|------|
| Tensile strength, dry | g./in.              | 336  |
| Tensile strength, wet | g./in.              | 205  |
| Elongation, wet       | percent             | 18   |
| Sheet weight          | g./ft. <sup>2</sup> | 6.90 |
| Tobacco content       | percent             | 83   |

These sheets were successfully wrapped on cigarillos to produce smoking articles of excellent taste, appearance, and burn odor.

#### Example IV

An attempt was made to prepare a polyester from suberic acid and glycerol by the procedure of Example III. The product was an alkyd resin which was insoluble in all common organic solvents. Likewise, the products of condensation of adipic acid or succinic acid with glycerol were insoluble polymers.

To illustrate means of overcoming this difficulty, a polyester was prepared from suberic acid (0.75 moles), azelaic acid (2.0 moles), and glycerol (1.0 moles) by the procedure of Example I. The product was soluble in a mixture of methanol and benzene, or in methanol or ethanol alone. Sheets were prepared from a 27% methanol slurry with a composition similar to those of Example III (10 parts ethylcellulose: 2 parts polyester: 60 parts tobacco), and after drying in air had the following properties:

|                       |                     |      |
|-----------------------|---------------------|------|
| Tensile strength, dry | g./in.              | 360  |
| Tensile strength, wet | g./in.              | 257  |
| Elongation, wet       | percent             | 17   |
| Sheet weight          | g./ft. <sup>2</sup> | 6.20 |
| Tobacco content       | percent             | 83   |

It will be noted that the addition of suberic acid, a shorter-chain dicarboxylic acid, to the reaction mixture resulted in a polyester which substantially improved the sheet tensile properties over those obtainable with azelaic acid alone. This sheet was also successfully wrapped on cigarillos to produce smoking articles of good quality and appearance.

#### Example V

To illustrate the effect of increasing the polyester content of tobacco sheets, the polyester of Example IV was incorporated into a 30% methanol slurry containing 10 parts of ethylcellulose, 3.3 parts of polyester, and 44.4 parts of tobacco. Sheets cast from this mixture had the following properties:

|                       |                     |      |
|-----------------------|---------------------|------|
| Tensile strength, dry | g./in.              | 806  |
| Tensile strength, wet | g./in.              | 550  |
| Elongation, wet       | percent             | 22   |
| Sheet weight          | g./ft. <sup>2</sup> | 8.85 |
| Tobacco content       | percent             | 77   |

These sheets had enough stretch to be wrapped successfully on large (Perfecto) cigars to produce smoking articles of excellent quality and appearance. It is apparent from the sheet properties that tensile strength and elongation are improved by increasing the amount of polyester and reducing tobacco content.

#### Example VI

To illustrate the effect of increasing the amount of suberic acid in the polyester of Example IV, a similar product was prepared by the same procedure from suberic acid (1.25 moles), azelaic acid (1.5 moles), and glycerol (1.0 mole) in benzene solution. This material was also soluble in polar solvents, in contrast to the alkyd resin obtained from suberic acid alone.

Sheets were prepared with the same compositions as those of Examples IV and V, but incorporating the new polyester of this example in place of that of Example IV. The 10 parts adhesive: 2 parts polyester: 60 parts tobacco formulation produced a sheet with the following properties using a methanol solvent:

|                       |                     |      |
|-----------------------|---------------------|------|
| Tensile strength, dry | g./in.              | 428  |
| Tensile strength, wet | g./in.              | 255  |
| Elongation, wet       | percent             | 18   |
| Sheet weight          | g./ft. <sup>2</sup> | 6.36 |
| Tobacco content       | percent             | 83   |

It is evident that the dry tensile strength increases with further additions of suberic acid, but that there is essentially no increase in wet tensile strength or elongation. These sheets were also successfully wrapped on cigarillos to produce smoking articles of good quality and appearance.

The sheets with the 10 parts adhesive: 3.3 parts polyester: 44.4 parts tobacco formulation, corresponding to those of Example V, had the following properties:

|                       |                     |      |
|-----------------------|---------------------|------|
| Tensile strength, dry | g./in.              | 714  |
| Tensile strength, wet | g./in.              | 475  |
| Elongation, wet       | percent             | 18   |
| Sheet weight          | g./ft. <sup>2</sup> | 6.68 |
| Tobacco content       | percent             | 77   |

Again there is no improvement in tensile strength or elongation over the sheets containing lesser amounts of suberic acid. This material made a satisfactory filler for cigarettes and also smoked well in a pipe.

#### Example VII

To illustrate the successful use of adipic acid in this invention a polyester was prepared from adipic acid (1.25 moles), azelaic acid (1.5 moles), and glycerol (1.0 mole) in benzene solution by the procedure of Example I. A sheet with the composition of Example IV was prepared with this polyester in methanol and had the following properties:

|                       |                     |      |
|-----------------------|---------------------|------|
| Tensile strength, dry | g./in.              | 375  |
| Tensile strength, wet | g./in.              | 230  |
| Elongation, wet       | percent             | 13   |
| Sheet weight          | g./ft. <sup>2</sup> | 6.45 |
| Tobacco content       | percent             | 77   |

It will be noted that addition of adipic acid to the reaction mixture produces a plasticizer with less favorable properties than that made with suberic acid. Nevertheless, this sheet could be wrapped on a cigarillo to give acceptable quality and appearance of the smoking article.

#### Example VIII

To illustrate the use of aliphatic triols other than glycerol, a polyester was prepared by the procedure of Example I from azelaic acid (2.75 moles) and 1,2,6-hexanetriol (1.0 mole) in benzene solution. A sheet with the formulation of Example V was cast with a 30% methanol slurry and had the following properties:

|                       |                     |      |
|-----------------------|---------------------|------|
| Tensile strength, dry | g./in.              | 430  |
| Tensile strength, wet | g./in.              | 340  |
| Elongation, wet       | percent             | 12   |
| Sheet weight          | g./ft. <sup>2</sup> | 5.95 |
| Tobacco content       | percent             | 77   |

This sheet was wrapped on a cigarillo to produce a smoking article of acceptable quality and appearance.

#### Example IX

A series of polyesters was prepared from glycerol (1.0 mole) and varying amounts of azelaic acid by the procedure of Example III. It was found that when less than two moles of azelaic acid were combined with the glycerol an insoluble alkyd resin was obtained. When two

or more moles of azelaic acid were employed in the condensation the polyester was soluble in organic solvents, such as benzene, toluene, and methanol. These soluble polyesters were used to prepare tobacco sheets with the formulation of Example V (77% tobacco). The following data were obtained from the sheets.

| Azelaic Acid, Moles | Tensile Strength, Dry g./in. | Tensile Strength, Wet g./in. | Elong., Wet, Percent | Sheet Weight g./ft. <sup>2</sup> |
|---------------------|------------------------------|------------------------------|----------------------|----------------------------------|
| 2.00                | 483                          | 333                          | 23                   | 6.15                             |
| 2.25                | 415                          | 283                          | 28                   | 6.10                             |
| 2.50                | 465                          | 283                          | 20                   | 6.60                             |
| 2.75                | 465                          | 255                          | 28                   | 6.31                             |
| 3.00                | 400                          | 235                          | 26                   | 5.85                             |

All of these sheets could be wrapped successfully on large (Perfecto) cigars. The optimum combination of good physical properties and pleasant burn odor is at about a 2.75/1.00 mole ratio of azelaic acid to glycerol.

#### Example X

As an illustration of the wide range in physical properties obtainable with the polyesters of this invention, the plasticizer of Example III was employed in a number of different formulations with methanol with tobacco contents ranging between 70 and 83%. In one case, A, a humectant (triethylene glycol) was added to obtain increased flexibility and stable high water content. The formulations and sheet data are presented in the following table:

| Sheet.....                              | A    | B    | C    | D    | E    |
|-----------------------------------------|------|------|------|------|------|
| Ethylecellulose, parts.....             | 10   | 10   | 10   | 10   | 10   |
| Polyester, parts.....                   | 4    | 4    | 2    | 2.5  | 2    |
| Tobacco, parts.....                     | 40   | 40   | 40   | 50   | 60   |
| Humectant, parts.....                   | 0.33 |      |      |      |      |
| Tobacco content, percent.....           | 70   | 74   | 77   | 80   | 83   |
| Tensile strength, dry, g./in.....       | 312  | 480  | 475  | 625  | 336  |
| Tensile strength, wet, g./in.....       | 258  | 275  | 282  | 276  | 205  |
| Elongation, dry, percent.....           | 27   | 10   | 9    | 10   | 6    |
| Elongation, wet, percent.....           | 40   | 30   | 20   | 24   | 18   |
| Sheet weight, g./ft. <sup>2</sup> ..... | 4.35 | 4.85 | 4.45 | 5.59 | 6.90 |

Sheet A could be wrapped successfully on a big cigar or cigarillo even when air-dried and stored at 80% relative humidity without remoistening, due to the water retained in the sheet by the humectant. Sheets B, C, and D could be wrapped successfully on a big cigar or cigarillo after spraying with water. Sheet E could not be wrapped on a big cigar, but was still flexible enough to be applied as cigarillo wrapper. All of these smoking articles had good appearance, taste, and burn odor.

#### Example XI

A polyester was prepared from glutaric acid (2.75 moles) and glycerol (1.0 mole) by the procedure of Example I. This was incorporated into a tobacco sheet with the formulation of Example V using methanol, and the following sheet data were obtained:

|                             |                     |      |
|-----------------------------|---------------------|------|
| Tensile strength, dry ..... | g./in.              | 639  |
| Tensile strength, wet ..... | g./in.              | 482  |
| Elongation, wet .....       | percent             | 18   |
| Sheet weight .....          | g./ft. <sup>2</sup> | 6.20 |
| Tobacco content .....       | percent             | 77   |

This sheet could be wrapped successfully on cigarillos to yield smoking articles of acceptable quality and appearance.

#### Example XII

A polyester was prepared from sebacic acid (2.75 moles) and glycerol (1.0 mole) by the procedure of Example I. This was incorporated into a tobacco sheet with the formulation of Example V, and the following sheet data were obtained:

|                             |                     |      |
|-----------------------------|---------------------|------|
| Tensile strength, dry ..... | g./in.              | 447  |
| Tensile strength, wet ..... | g./in.              | 299  |
| Elongation, wet .....       | percent             | 25   |
| Sheet weight .....          | g./ft. <sup>2</sup> | 6.20 |
| Tobacco content .....       | percent             | 77   |

A second sheet was prepared from the same polyester (2.5 parts) with 10 parts of ethylamyllose and 50 parts of tobacco in benzene. These sheets had the following properties:

|                             |                     |      |
|-----------------------------|---------------------|------|
| Tensile strength, dry ..... | g./in.              | 350  |
| Tensile strength, wet ..... | g./in.              | 215  |
| Elongation, wet .....       | percent             | 18   |
| Sheet weight .....          | g./ft. <sup>2</sup> | 5.95 |
| Tobacco content .....       | percent             | 80   |

Both types of sheet could be wrapped successfully on cigarillos to produce articles of acceptable quality and appearance.

The auxiliary plasticizer-adhesives of this invention can be incorporated into a tobacco product such as a sheet in the manner described above to produce the beneficial plasticizing effect necessary to make cigar wrappers which can be fed automatically from a bobbin to a cigar machine. Generally, flavoring and coloring materials, humectant, and other inert ingredients such as ash improvers are incorporated into cigar wrapper sheet. Cigars and cigarillos prepared from tobacco sheet wrapper of this invention are light in color, smooth in texture, uniform in quality, inexpensive, and do not dissolve or disintegrate in the mouth when wet with saliva. The same type of tobacco sheet, containing the plasticizers of this invention, may also be used as cigar binder or as a filler in the form of strands or filaments, which may be chopped, in other smoking articles such as cigarillos, little cigars, pipes or cigarettes. Some modification in sheet weight and in the proportions of the various ingredients employed may be used for the various applications mentioned.

The tobacco products of this invention generally contain more than two thirds by weight of tobacco and may contain four fifths or more tobacco. Not only finely divided tobacco, but fibers from tobacco and other materials may be used. The polyester materials generally make up less than one eighth of the product and are preferably used in the range of 2-8% by weight. Other ingredients include some moisture, the adhesive and ash control materials.

Tobacco products may be made from the novel compositions of this invention by extrusion, casting, spraying or dip coating with a slurry of the ingredients in a solvent; or tobacco dust may be coated onto the wet solvent preparation of adhesive and polyester.

What is claimed is:

1. A method of making a smoking product comprising in combination the steps of forming a polysaccharide derivative solution in an organic liquid, adding thereto a polyester derived from a dicarboxylic acid and an aliphatic triol, and mixing therein a quantity of finely divided tobacco equal to at least twice the combined weight of the polysaccharide and polyester, to form a viscous slurry, shaping said slurry and evaporating the organic liquid therefrom.
2. A method of making a smoking product comprising in combination the steps of forming a wet surface from an organic liquid containing in solution a polysaccharide derivative and a polyester derived from a dicarboxylic acid and an aliphatic triol, coating said wet surface with finely divided tobacco to form a composition of matter

and evaporating said liquid from said composition to form a smoking product.

3. A method according to claim 1 in which the slurry is shaped into a sheet.

4. A method according to claim 1 in which the slurry 5 is extruded.

5. A method according to claim 4 in which the slurry is extruded as a filament.

6. A method according to claim 3 in which the sheet is formed on a casting surface.

## References Cited in the file of this patent

## UNITED STATES PATENTS

|           |                    |               |
|-----------|--------------------|---------------|
| 2,348,324 | Bond               | May 9, 1944   |
| 2,734,510 | Hungerford et al.  | Feb. 14, 1956 |
| 2,734,513 | Hungerford et al.  | Feb. 14, 1956 |
| 2,739,599 | Abbott             | Mar. 27, 1956 |
| 2,747,583 | Frankenburg et al. | May 29, 1956  |
| 2,755,207 | Frankenburg        | July 17, 1956 |